

April 23, 1935.

G. BENEDETTO

1,999,077

PROCESS OF MAKING METAL ROAD STUDS

Filed June 11, 1934

Fig. 1.



Fig. 3.



Fig. 2.



Fig. 4.



Fig. 5.



Inventor

Giuseppe Benedetto

22 By  
22 Station, Corl, Morse & Grindle  
Attorneys

## UNITED STATES PATENT OFFICE

1,999,077

## PROCESS OF MAKING METAL ROAD STUDS

Giuseppe Benedetto, Novara, Italy, assignor to  
Omes Holding Company Limited, London, Eng-  
land, a British company

Application June 11, 1934, Serial No. 730,110  
In Great Britain June 6, 1933

2 Claims. (Cl. 29—148)

This invention comprises improvements in the process of forming metal studs which are frequently embedded in the surface of roads for the purpose of affording guidance to traffic as to the lines along which it may proceed.

Hitherto metal blocks or studs let into the surface of the road have been constructed of cast metal or of stainless steel, but stainless steel studs produced by ordinary casting or forging operations are expensive and metal castings are bulky and difficult to fix.

The present invention deals particularly with the formation of a road stud having the form of a large flattened head portion and a stem integral therewith projecting downwardly from the underside of the head portion so as to enter into the material of the road.

Further, according to the present invention a method of making a road stud consists in taking a bar of metal of a diameter equal to that desired for a stem portion and forming a broad flat head on the end thereof by forging in an electrical upsetting machine, preferably with subsequent pressing in a die-stamp.

The accompanying drawing illustrates by way of example various kinds of studs in accordance with the present invention, and in the drawing:—

Figure 1 is a side elevation of one form of stud;

Figure 2 is a perspective view of the same stud upside down to show the underside;

Figure 3 is a side elevation of a second form;

Figure 4 is a view similar to Figure 2 of the form shown in Figure 3, and

Figure 5 is a perspective view of the upper side of a third form of stud.

Referring to Figures 1 and 2 the stud comprises a stem 11 and a broad flat head 12 square as viewed in plan and convex on its upper side. The underside is concave as indicated at 13 and is provided with four downwardly projecting studs or nibs 14 which are intended to enter the road surface and prevent the head from turning relatively thereto about the stem 11.

Referring to Figures 3 and 4, these show a stud having a stem 15 and a convex circular head 16, the underside of which is hollow as shown at 17 and provided with radial ribs 18 which not only stiffen the convex head portion but also serve to key the stud against rotation relatively to the road surface. In addition the stem 15 is split and splayed at its bottom end by cutting it longitudinally in a shearing machine for a certain distance, resulting in two inclined portions 19 similar to the end of a rag-bolt. These afford an

additional key against rotation or lifting of the stud.

Figure 5 illustrates a stud comprising a three-cornered head portion 20 on a stem 21 the bottom end of which is split and splayed at 22 as already described. In the centre of the head portion there is an embossed letter 23. Studs of this kind can be set in a road surface so that they point towards a parking place and lead the motorist to the entrance thereof. Conveniently such 10 studs may be formed from metal of a distinctive colour, such as bronze.

The method of manufacture of the studs illustrated may comprise first taking a bar of a diameter equal to that of the stem of the stud, then 15 upsetting (in an electrical forging machine such, for example, as that described in prior United States Patent No. 1,878,810) a head containing a sufficiency of metal to constitute the head of the finished stud and finally shaping this head 20 in a die- or drop-stamp while the metal is still hot from the electric forging operation. The amount of metal in the head may be as much as corresponds to about fifteen diameters of the stem. If steel is employed it is preferable to use 25 stainless steel. The head can then be polished after forging.

It will be observed that by following the procedure outlined in my prior patent referred to, the stud is formed to provide a dense forged 30 structure in which the grain runs longitudinally along the shank and is bent round in the head so that the fibre of the metal extends parallel with the upper and lower surfaces. If one of the road studs, manufactured as described in my prior 35 patent, be cut in half and the sectioned surface be etched with acid the lines of flow of the metal will be seen to follow the course just described. This is due to the method of forging, and results in a stud much more durable and stronger 40 than those produced by casting. Thus the fibre of the metal lies parallel to the upper surface of the stud and takes the wear in traffic. At the same time the method of forging adopted permits the production of downward projections 45 from the underside of the head into which the metal is caused to flow by the stamping operation, the fibre of the metal again extending parallel to the length of the projections or ribs to lend 50 additional strength thereto.

Alternatively non-ferrous metal such as aluminium or copper or alloys of aluminium or copper may be employed; the alloys may include brass, Monel metal, bronzes in general or other 55

alloys of copper with tin, nickel, aluminium or zinc.

A convenient diameter of stem using a non-ferrous metal is  $\frac{1}{8}$ ths of an inch diameter and the head may be conveniently about four inches across. Instead of splitting and splaying the bottom end of the stem a head may be upset thereon if desired and then flattened in a plane parallel to the stem.

10 I claim:—

1. A method of making road studs which comprises forming on one end of a bar of non-ferrous metal of a diameter equal to that desired for a stem portion, a broad flat head by first heating the end of the bar and applying pressure thereto in the direction of the length of the bar, whereby the grain in the head of the stud may extend generally radially and the grain in the stem may extend generally longitudinally, sub-

sequently pressing the head to final shape in a die stamp, and deforming a portion of the stem spaced from the head to increase a lateral dimension of such portion.

2. A method of making road studs which comprises forming on one end of a bar of metal of a diameter equal to that desired for a stem portion, a broad flat head by first heating the end of the bar by the passage therethrough of electric current and simultaneously applying pressure thereto in the direction of the length of the bar, whereby the grain in the head of the stud may extend generally radially and the grain in the stem may extend generally longitudinally, subsequently pressing the head to final shape in a die stamp, and splitting and splaying that end of the stem remote from the head to increase a lateral dimension thereof.

GIUSEPPE BENEDETTO.